

1,342,282.

M. W. GLEASON.

LAMINATED GLASS.

APPLICATION FILED JUNE 10, 1919.

Patented June 1, 1920.

Fig. 1.



Fig. 2.



Fig. 3.



WITNESSES

George Maylor  
Josh. Beeler

INVENTOR

M. W. Gleason  
BY M. M. Co.  
ATTORNEYS

# UNITED STATES PATENT OFFICE.

MARSHALL W. GLEASON, OF BROOKLYN, NEW YORK, ASSIGNOR TO GLEASON TIEBOUT  
GLASS CO., OF NEW YORK, N. Y., A CORPORATION OF NEW YORK.

## LAMINATED GLASS.

1,342,282.

Specification of Letters Patent.

Patented June 1, 1920.

Application filed June 10, 1919. Serial No. 303,182.

*To all whom it may concern:*

Be it known that I, MARSHALL W. GLEASON, a citizen of the United States, and a resident of the city of New York, borough 5 of Brooklyn, in the county of Kings and State of New York, have invented a new and Improved Laminated Glass, of which the following is a full, clear, and exact description.

10 This invention relates to plastic or vitreous matter and has particular reference to the method or means for making such compositions of matter in laminated form having among other things the following 15 characteristics and structural advantages; first, the construction of vitreous objects such as globes for electric lamps or the like in which there are provided a plurality of layers or laminæ of any suitable or varying 20 tints or colors and with the different laminæ so assembled or united that each of the laminæ loses its individual color or character in blending with the others; secondly, the assemblage of laminated glass- 25 ware or the like in such a manner that the strength of the article is very much increased over a single layer structure of the same or greater thickness, and thirdly, the provision of a glass globe or reflector, having on its inner surface a thin tinted layer which has the function of filtering out 30 from the light certain tints or colors so as to produce a light very similar to natural daylight.

35 With the foregoing and other objects in view my invention comprises features of construction hereinafter more specifically described and illustrated in the accompanying drawings, of which—

40 Figure 1 is a side elevation of a lamp globe made in accordance with this invention and illustrating one of its many uses.

Fig. 2 is an enlarged sectional view illustrating the laminated form of this structure; and

45 Fig. 3 is a fragmentary inside view of the same, certain portions of the laminæ being broken away to show others.

Referring now more specifically to the drawings I show a plastic structure comprising a plurality of laminæ the same being made into the form of a globe and used in connection with electric lights or the like. Of the laminæ the innermost layer 10 is 50 relatively thin and of a distinct tint such as

blue, though being of so thin a nature and the color being so relatively mild the structure is not materially altered in its appearance because of the colored layer, except as the light is modified by it in passing through 60 it as will more fully appear hereinafter.

The outermost layer 11 is clear and colorless and is materially thicker than the innermost layer.

65 The intermediate layer 12 is of a neutral character as to color and may be termed white or opal. This layer is preferably of approximately the same thickness as the outermost layer 11.

A piece of glassware made in accordance 70 with this invention possesses phenomenal strength because the strength of an article of plastic material or the like depends upon the extent of its surface. In the making of this glass in which there are three layers 75 united to one another there is in effect a condition involving three times as many surfaces as if a single ply or layer of glass were present. The molten glass from which the several laminæ are formed is assembled by the blower dipping first his blow- pipe into the blue glass then into the opal and then into the clear glass. By the exercise of skill and experience he gathers the proper proportions of the different species 80 of glass upon the end of his blow-pipe forming a solid mass of blue, white, and clear respectively. He then blows through the pipe for the purpose of enlarging or expanding the mass and finally plunges it 85 into a suitable mold for the purpose of giving the mass the proper shape. The several layers or laminæ are thus spread evenly throughout the configuration. The several laminæ though united each to each 90 firmly do not blend or mix with one another.

95 In the practice of this invention I do not wish to be limited to any particular tints or colors of the glass comprising the several 100 laminæ but for the purposes set forth I employ blue for the innermost layer and neutral characters for the others. The blue layer filters out from the light given off by the electric light the excess red and yellow 105 rays whereby there is produced a most satisfactory approximation of artificial day light due to the combination of the thin blue layer and the thicker opal or neutral layer. The clear layer on the outside af- 110

fords sufficient body and added strength to the structure but without decreasing the translucency of the medium.

I claim:

- 5 1. The herein described article of glass-ware comprising a plurality of laminæ one of which is of distinctive color while the others are of a neutral character as to color but different from each other.
- 10 2. The herein described article of glass-ware in the form of a hollow globe whose shell is composed of a plurality of laminæ

the innermost of which is of a distinctive color, the outermost of which is clear, while the intermediate layer is of a translucent 15 nature with a neutral tint.

3. The herein described article of glass-ware composed of a plurality of laminæ, the innermost of which is relatively thin and of a bluish color, the outermost of 20 which is clear, and the intermediate layer of which is of a translucent nature.

MARSHALL W. GLEASON.